

Patented May 1, 1951

2,551,091

# UNITED STATES PATENT OFFICE

2,551,091

## PROCESS FOR COLOR DEVELOPING, INCLUDING TREATMENT WITH A QUATERNARY AMMONIUM SALT

Vernon William Blanchard, South River, N. J., assignor to E. I. du Pont de Nemours and Company, Wilmington, Del., a corporation of Delaware

No Drawing. Application September 14, 1949, Serial No. 115,769

6 Claims. (Cl. 95—88)

1

This invention relates to processes of color photography. More particularly it relates to a process for modifying the color of quinoneimine and/or azomethine dye images obtained from the color coupling development of immobile color formers containing a sulfonamide or carbonamide group having a hydrogen atom attached to the amino-nitrogen atom in photographic elements. Still more particularly it relates to a process of treating an exposed photographic element which contains an immobile color former containing a carbonamide or sulfonamide group having a hydrogen atom attached to the amido-nitrogen atom after exposure but prior to completion of aqueous processing. Still more particularly it relates to such processes wherein a surface-active quaternary ammonium compound is used in the aqueous treating bath.

An object of this invention is to improve the color of the quinoneimine or azomethine dye image or images obtained from color formers of the above type which are disposed in a layer of a photographic element. A further object is to provide a simple and economical but yet effective method of varying the color of such quinoneimine or azomethine dye images. Still other objects will be apparent from the following description of the invention.

It has been found that the color of a quinoneimine or azomethine dye image formed by the color coupling development of a colloid silver halide emulsion layer group photographic element can be modified by treating an element which contains or contained an immobile color former containing a carbonamide or sulfonamide group having a hydrogen atom attached to the amido-nitrogen atom disposed in, or constituting a water-permeable colloid layer, after exposure, in an aqueous treating solution containing a small amount of a surface-active quaternary ammonium salt having an aliphatic hydrocarbon radical of 8 to 22 carbon atoms attached to the pentavalent nitrogen atom.

The aqueous treating solution containing such salts may be applied at any stage in the processing of the exposed film to a dye image e. g., prior to, during or subsequent to development. The salts are preferably used in the aqueous alkaline developer solution. The amount of quaternary ammonium salt used in the aqueous treating bath can be varied over a fairly wide range, but in general, from 0.2 gram to 25 grams per liter of solution is sufficient to make a significant change in the color of the dye image.

While the invention is useful with any immobile color former containing a primary carbonamide group or a primary sulfonamide group it is especially useful with color former amidobenz-

2

aldehyde acetals of hydroxyl polymers containing a plurality of recurring intralinear



5 groups. The color former units of the polymer may be represented by the formula:

10



15

wherein the free bonds are attached to the other chain units e. g.,



groups. R is a color former nucleus which is joined directly to X or through a hydrocarbon 20 radical, X is



25

or  $-\text{SO}_2-$ . R may be a pyrazolone, phenol, naphthol or acylacet nucleus. A relatively large number of such color formers are known to the art. Some are described in U. S. Patents 2,810,943, 2,320,422, 2,380,032, 2,380,033, 2,397,864, 2,423,572, 2,464,597, 2,465,067. Still others are described in 30 assignee's copending applications Serial Nos. 9,330, filed February 18, 1948, now Patent No. 2,513,190 and 19,155, filed April 5, 1948, now Patent No. 2,489,655.

35

It has been found, for example, that the magenta azomethine dyes which are formed from a polyvinyl acetal color former containing the following color former nuclei which are attached to a polyvinyl alcohol chain by an acetal linkage are especially beneficially improved in color by 40 the foregoing treatment:

45



(I)

50



(II)

The color change consists in a narrowing and shifting of the green absorption band and an increase in the red and blue transmission. The changes improve the spectral characteristics of the dyes in that the final colors more closely approximate the ideal magenta color that is desired for uses in processes of subtractive color photography.

While the color changes are particularly advantageous with the above types of magenta color formers, a marked improvement in a cyan or blue-green quinoneimine dye from a polyvinyl acetal color former containing recurring units of Formula III may be obtained by a similar treatment.



As previously stated, it is preferred to have the quaternary ammonium salts in the color developer solutions. The latter solutions may be any of the conventional types and contain a color developing agent having an unsubstituted amino ( $\text{NH}_2$ ) group such as phenylene diamine and its N-monoalkyl and N-diethyl substitution products containing from 1 to 4 carbon atoms in the alkyl group of which p-diethylaminoaniline is the preferred agent. These color developing agents are usually used in the form of their water-soluble salts since the latter are more stable and are more easily dissolved. Suitable salts are the hydrochloride, sulphate and chloracetate. The developer solutions moreover, may contain the usual water-soluble sulfites, e. g., sodium, potassium, and ammonium sulfite and alkalies, e. g., sodium carbonate, ammonium hydroxide and sodium metaborate and other developer constituents.

The invention will be further illustrated but is not intended to be limited by the following examples wherein the parts stated are by weight unless otherwise indicated.

#### Example I

A cellulose acetate film base bearing a layer composed of light sensitive silver salts dispersed in a polyvinylacetal containing color former units of Formula II above was exposed and developed for 10 minutes at 68° F. in a solution made by admixing the following ingredients:

|                                                   |       |       |
|---------------------------------------------------|-------|-------|
| p-Aminodiethylaniline.HCl                         | grams | 2.5   |
| $\text{Na}_2\text{SO}_3$ (desiccated)             | do    | 10.0  |
| $\text{Na}_2\text{CO}_3 \cdot \text{H}_2\text{O}$ | do    | 29.25 |
| KBr                                               | do    | 2.00  |
| Water to                                          | liter | 1     |

The film was washed in water for 2 minutes, fixed at 68° F. for 5 minutes in a solution made by adding 200 grams of desiccated sodium hyposulfite in one liter of water, washed 10 minutes, bleached 5 minutes in a bath of the formula:

|                                    |       |    |
|------------------------------------|-------|----|
| $\text{K}_3\text{Fe}(\text{CN})_6$ | grams | 60 |
| Boric acid                         | do    | 10 |
| Borax                              | do    | 5  |
| Water to                           | liter | 1  |

washed 2 minutes, fixed 5 minutes in a solution made by admixing the following ingredients:

|                      |       |     |
|----------------------|-------|-----|
| Ammonium thiocyanate | grams | 100 |
| Borax                | do    | 50  |
| Water to             | liter | 1   |

washed in water for 15 minutes and dried. A strip of the film was then soaked for 5 minutes in a 0.1% aqueous solution of a mixture of long chain alkyl trimethyl ammonium bromide where in the alkyl groups contained from 8 to 18 carbon atoms and correspond to such groups in the higher alcohols obtained from the hydrogenation of cocoanut oil. The color of the dye image obtained was markedly changed as compared with a second strip of the film which was not given the latter treatment, there being a shift in the green absorption band and an increase in the red and blue transmission.

A third strip was soaked in a similar bath containing, in addition to the surface active ammonium salts, 3% of sodium carbonate. The color change was similar to the first strip.

Upon soaking the first and third strips in an aqueous solution containing 0.5% of a mixture 20 of alkyl sulfates of 10 to 18 carbon atoms the color changed back to approximately the color of the second strip.

#### Example II

25 A photographic film element bearing a layer composed of light-sensitive silver salts dispersed in the polyvinyl acetal color former of Formula I above was exposed to an object field and then processed as follows:

30 1. Developed for ten minutes at 68° F. in a color developing solution made by admixing the following components:

|                                                   |       |       |
|---------------------------------------------------|-------|-------|
| p-Aminodiethyl aniline.HCl                        | grams | 2.50  |
| $\text{Na}_2\text{SO}_3$ (desiccated)             | do    | 10.00 |
| $\text{Na}_2\text{CO}_3 \cdot \text{H}_2\text{O}$ | do    | 29.25 |
| KBr                                               | do    | 2.00  |
| Cetyl pyridinium bromide (A)                      | do    | 5.00  |
| Water to                                          | liter | 1     |

40 2. Washed in water for three minutes;

3. Fixed at 68° F. for ten minutes in a solution made by admixing the following ingredients:

|                    |       |     |
|--------------------|-------|-----|
| Sodium thiosulfate | grams | 200 |
| Water to           | liter | 1   |

45 4. Washed in water for 15 minutes;

5. Bleached for five minutes at 68° F. in a solution made by admixing the following ingredients:

|                                    |       |    |
|------------------------------------|-------|----|
| $\text{K}_3\text{Fe}(\text{CN})_6$ | grams | 60 |
| Boric acid                         | do    | 10 |
| Borax                              | do    | 5  |
| Water to                           | liter | 1  |

55 6. Washed for two minutes in water;

7. Fixed for five minutes at 68° F. in a solution made by admixing the following ingredients:

|                      |       |     |
|----------------------|-------|-----|
| Ammonium thiocyanate | grams | 100 |
| Borax                | do    | 50  |
| Water to             | liter | 1   |

60 8. Washed for a period of 15 minutes in water and dried.

In the above procedure, a control film was 65 treated in exactly the same way except that the cetyl pyridinium bromide was omitted from the developer solution.

Similar film elements but containing the color formers having units of Formulae II and III above 70 were treated in like manner and with developer solutions containing in place of cetyl pyridinium bromide (A), 5 cc. per liter of alkyl dimethyl benzyl ammonium chloride (10% aqueous solution) (B), 5 grams per liter of octadecyl trimethyl ammonium bromide (C), 5 cc. per liter

of diisobutyl phenoxy ethoxy ethyl dimethyl benzyl ammonium chloride (25% aqueous solution) (D), and 5 cc. per liter of the quaternary ammonium salt (20% aqueous solution) of Example I (E) with the results given in the following table as compared with control films not treated with the quaternary ammonium salts.

monium bromide, octadecyl trimethyl ammonium iodide, cetyl trimethyl ammonium iodide, cetyl triethyl ammonium iodide, cetyl triethyl ammonium bromide, cetyl benzyl diethyl ammonium chloride, eicosyl trimethyl ammonium bromide, docosyl trimethyl ammonium iodide, cetyl benzyl dimethyl ammonium chloride, octadecyl tri-

| Wave-length in<br>Milli-<br>microns | Film<br>Treatment | None | Density Readings <sup>1</sup> |      |      |      |      |                 |      |      |      |      |                     |      |      |      |
|-------------------------------------|-------------------|------|-------------------------------|------|------|------|------|-----------------|------|------|------|------|---------------------|------|------|------|
|                                     |                   |      | Color Former I                |      |      |      |      | Color Former II |      |      |      |      | Color Former<br>III |      |      |      |
|                                     |                   |      | A                             | B    | C    | D    | E    | None            | A    | B    | C    | D    | E                   | None | E    |      |
| 400                                 |                   |      | .32                           | .22  | .14  | .25  | .18  | .20             | .34  | .26  | .24  | .27  | .26                 | .28  | .35  | .36  |
| 440                                 |                   |      | .70                           | .60  | .54  | .68  | .56  | .60             | .54  | .48  | .46  | .49  | .50                 | .50  | .21  | .22  |
| 450                                 |                   |      | .72                           | .63  | .56  | .68  | .58  | .61             | .52  | .46  | .45  | .47  | .51                 | .51  | .17  | .17  |
| 460                                 |                   |      | .70                           | .61  | .54  | .67  | .55  | .59             | .50  | .44  | .44  | .45  | .47                 | .47  | .13  | .13  |
| 500                                 |                   |      | 1.20                          | 1.20 | 1.16 | 1.28 | 1.13 | 1.19            | 1.01 | 1.01 | 1.00 | .97  | 1.00                | 1.02 | .07  | .07  |
| 530                                 |                   |      | 1.49                          | 1.48 | 1.44 | 1.53 | 1.48 | 1.48            | 1.51 | 1.48 | 1.45 | 1.48 | 1.52                | 1.50 | .10  | .09  |
| 540                                 |                   |      | 1.51                          | 1.48 | 1.44 | 1.54 | 1.49 | 1.49            | 1.56 | 1.51 | 1.47 | 1.54 | 1.57                | 1.53 | .12  | .11  |
| 550                                 |                   |      | 1.50                          | 1.43 | 1.38 | 1.50 | 1.45 | 1.46            | 1.57 | 1.49 | 1.43 | 1.54 | 1.53                | 1.49 | .19  | .15  |
| 600                                 |                   |      | .85                           | .68  | .56  | .76  | .66  | .69             | .78  | .58  | .49  | .71  | .55                 | .54  | .85  | .65  |
| 650                                 |                   |      | .34                           | .24  | .14  | .26  | .19  | .23             | .28  | .17  | .15  | .21  | .17                 | .17  | 1.38 | 1.33 |
| 700                                 |                   |      | .19                           | .12  | .04  | .12  | .08  | .11             | .14  | .07  | .07  | .08  | .08                 | .10  | 1.45 | 1.46 |

<sup>1</sup> Taken from the density curves run on the General Electric Company spectrophotometer (described in the Journal of the Optical Society of America, vol. 25, pp. 305-311 (1935)).

### Example III

A multilayer having the following strata, in order, on a transparent support:

1. A silver halide emulsion layer for color development of a cyan image containing a color-former amido acetal of polyvinyl alcohol having several units of Formula III and sensitized for red light.
2. A thin, colorless separator layer of a hydrophilic hydrolyzed ethylene/vinyl acetate interpolymer.
3. An emulsion layer for color development of a yellow image containing a color-former amido acetal of polyvinyl alcohol and containing several units of the formula:



and sensitized for green light.

4. A separator layer like 2.
5. An emulsion layer for color development of a magenta image containing a color-former amido acetal of a polyvinyl alcohol containing several units of formula I and containing a yellow filter dye, e. g., Tartrazine (Colour Index No. 640), was exposed on a sector wheel sensitometer where each step is double the exposure of the preceding step and through three red, green and blue primary filters and color developed, washed, fixed, washed, bleached, fixed and washed after the manner described in Example II and then soaked for five minutes in a 0.125% aqueous solution of cetyl dimethyl benzyl ammonium chloride, washed and dried. The color of the dye image of each layer was changed, most significant was the increase of red and blue light transmission of the magenta layer and the increase of green light transmission of the cyan layer.

In place of the specific quaternary ammonium salts described in the foregoing examples, there may be substituted other specific salts of this type. Thus, there may be employed cetyl trimethyl ammonium bromide, dimethyl dicetyl am-

methyl ammonium methosulphate, decyl trimethyl ammonium iodide, cetyl cyclohexyl dimethyl ammonium bromide, dodecyl cyclohexyl dimethyl ammonium bromide, dodecyl trimethyl ammonium chloride, cetyl trimethyl ammonium chloride, octyl trimethyl ammonium iodide, octadecyl trimethyl ammonium bromide, dodecyl trimethyl ammonium bromide, octadecyl benzyl dimethyl ammonium chloride, cetyl triethanol dimethyl ammonium bromide, dodecyl ethanol dimethyl ammonium sulphate, etc.

- 30 40 While the above examples are all directed to the treatment of films of the type covered by U. S. Patent No. 2,397,864 the invention is not limited to such type. Similar films having the color formers of the above patents which are dispersed in various water-permeable colloid silver halide emulsions e. g., gelatin, casein, albumen, and the hydrolyzed ethylene/vinyl acetate copolymers of U. S. Patent No. 2,397,867 can be similarly treated. Likewise, films containing immobile color formers other than the polyvinyl acetal type can be used.
- 35 50 Suitable other color formers are immobile containing the carbonamide and sulfonamide groups of the above type are described in U. S. Patents 2,186,717, 2,356,475, 2,350,138, 2,319,426, 2,395,484, 2,397,867, and 2,435,629.
- 55 The invention can be used with elements wherein the color formers constitute or are disposed in a water permeable layer or stratum adjacent a light sensitive silver halide layer so that the silver halide grains are in coactive relationship with the color former. Elements of this type are described in U. S. Patents 2,363,764 and 2,350,380.
- 60 An advantage of the invention is that it provides an effective process for modifying color developed images in single or multilayer photographic elements. A further advantage is that it provides a simple and economical process for modifying the color of color developed images. A still further advantage is that the process is economical and utilizes commercially available quaternary salts. A further advantage is that it enables the photographic technician to correct the color of a dye image or images.
- 65 70 As many widely different embodiments of this invention can be made without departing from the spirit and scope thereof, it is to be under-

stood that the invention is not to be limited except as defined by the claims.

I claim:

1. In a process of producing a color developed dye image by exposing, color developing by a primary aromatic amine developing agent, bleaching and fixing a photographic film element bearing a light-sensitive silver halide layer having an immobile color former containing an amide group taken from the class consisting of carbonamide and sulfonamide groups which have a hydrogen atom attached to the amido-nitrogen atom in coactive relationship with the silver halide grains; the step which comprises treating the element after exposure in an aqueous treating bath containing 0.2 gram to 25.0 grams per liter of a quaternary ammonium salt the positive ion of which contains an aliphatic hydrocarbon radical having a chain of 8 to 22 carbon atoms.
2. In a process of producing a color developed dye image by exposing, color developing by a primary aromatic amine developing agent, fixing, bleaching and fixing a photographic film element bearing a light-sensitive silver halide layer having an immobile color former containing an amide group taken from the class consisting of carbonamide and sulfonamide groups which have a hydrogen atom attached to the amido-nitrogen atom in coactive relationship with the silver halide grains; the step which comprises treating the element after exposure in an aqueous treating bath containing from 0.2 gram to 25 grams per liter of a quaternary ammonium salt, the positive ion of which contains an alkyl radical having from 12 to 18 carbon atoms in a straight chain.
3. In a process of producing a color developed dye image by exposing, color developing by a primary aromatic amine developing agent, fixing, bleaching and fixing a photographic film element bearing a light-sensitive silver halide layer having an immobile polyvinyl acetal color former containing a primary carbonamide group which has a hydrogen atom attached to the amido-nitrogen atom in coactive relationship with the silver halide grains; the step which comprises treating the element after exposure in an aqueous treating bath containing from 0.2 gram to 25.0 grams per liter of a quaternary ammonium salt the positive ion of which contains an aliphatic hydrocarbon radical having a chain of 8 to 22 carbon atoms.
4. In a process of producing a color developed dye image by exposing, color developing by a primary aromatic amine developing agent, fixing, bleaching and fixing a photographic film element bearing a light-sensitive silver halide

layer having an immobile polyvinyl acetal color former containing a sulfonamide group which has a hydrogen atom attached to the amido-nitrogen atom in coactive relationship with the

5. silver halide grains; the step which comprises treating the element after exposure in an aqueous treating bath containing from 0.2 gram to 25.0 grams per liter of a quaternary ammonium salt the positive ion of which contains an aliphatic hydrocarbon radical having a chain of 8 to 22 carbon atoms.
6. In a process of producing a color developed dye image by exposing, color developing by a primary aromatic amine developing agent, fixing, bleaching and fixing a photographic film element bearing a light-sensitive silver halide layer having an immobile color former containing an amide group taken from the class consisting of carbonamide and sulfonamide groups which have a hydrogen atom attached to the amido-nitrogen atom in coactive relationship with the silver halide grains; the step which comprises developing the exposed element in an aqueous alkaline developing bath containing a
- 15 primary aromatic amino developing agent and from 0.2 gram to 25.0 grams per liter of a quaternary ammonium salt, the positive ion of which contains an aliphatic hydrocarbon radical having a chain of 8 to 22 carbon atoms.
- 20
- 25
- 30
- 35
- 40
- 45

VERNON WILLIAM BLANCHARD.

#### REFERENCES CITED

- 50 The following references are of record in the file of this patent:

#### UNITED STATES PATENTS

| Number    | Name      | Date          |
|-----------|-----------|---------------|
| 2,301,381 | Dickey    | Nov. 10, 1942 |
| 2,307,161 | Schneider | Jan. 5, 1943  |
| 2,376,141 | Henn      | May 15, 1945  |